

C. S. BIRD.

FLOOR COVERING.

APPLICATION FILED JAN. 30, 1913.

1,131,317.

Patented Mar. 9, 1915.



Witnesses

F. C. Curran

E. C. Murphy

Inventor,

Charles S. Bird

*By Henry J. Miller, atty.*

# UNITED STATES PATENT OFFICE.

CHARLES S. BIRD, OF EAST WALPOLE, MASSACHUSETTS.

## FLOOR-COVERING.

1,131,317.

Specification of Letters Patent. Patented Mar. 9, 1915.

Application filed January 30, 1913. Serial No. 745,257.

To all whom it may concern:

Be it known that I, CHARLES S. BIRD, of East Walpole, in the county of Norfolk and State of Massachusetts, have invented certain new and useful Improvements in Floor-Coverings, of which the following is a specification.

This invention has reference to improvements in floor coverings generally and more particularly to improvements in floor coverings treated with asphaltic or other waterproofing materials.

One object of the invention is to facilitate the manufacture of floor coverings having a backing of material to some extent waterproof by the use in said backing material of a constituent having the quality of becoming comparatively hard or, so called, chilled, within a short time of its application.

Another object of the invention is to so construct floor covering having a waterproofing and a backing that said backing will not tend to effect the softening of such waterproofing.

Still another object of the invention is to so construct floor covering comprising a base coated or saturated with asphaltic material and having a backing coating applied to said body in a fluid and preferably heated condition that the asphaltic material shall not be softened materially by the application of said backing.

Other objects of the invention will appear from the following description.

The invention consists in floor covering comprising a base or body of asphaltic material having a backing coating of wax.

The invention also consists in floor covering hereinafter described and claimed.

The drawing illustrates the improved floor covering in sectional view, the thickness of the various layers or coatings thereof being exaggerated.

Floor covering herein generally referred to includes any base or body formed from woven, granular or fibrous material having, after its formation, a backing coating adapted to resist wear to some extent and of a substantially waterproof nature.

In the manufacture of oil cloth and some kinds of linoleum it is usual, after the manufacture of the body or base to apply thereto a backing coating in the nature of a comparatively thick paint in which oil or other moisture resisting material is present whereby the back of said body or base is rendered

less liable to wear and by which moisture is, to some extent, excluded from said body or base. After the application of such backing coating it has heretofore been necessary to handle and store the material with extreme care by the assistance of expensive machinery to permit the backing coating to become perfectly dry, the delay occasioned by such drying operation amounting to periods of many hours. By the use of the material for such backing coating the expensive machinery may be dispensed with and the delay avoided as the new backing coating will become set or chilled within comparatively few seconds of its application.

In carrying this invention into practice I take a body or base 5 of fibrous material preferably of paper felt and saturate the same with asphaltic material. I then apply to one surface of such felt the coating of paint 6 and after such coating becomes sufficiently dry I print thereon a pattern coating 7 of paint considerably thicker than the coating 6 whereby an upper wearing surface is provided. After this pattern or wearing coating 7 becomes dry I apply to the back of the base 5 the coating 8 of Montan wax so called.

Referring now to the floor covering more specifically mentioned above, it has been found that a very durable and satisfactory floor covering may be made by taking a sheet or web of comparatively thick felt, usually made of stock from which paper is made and having considerable elasticity by reason of its fibrous nature. Great difficulty has, however, been encountered in providing for the protection of this felted fibrous base or body from moisture and it has been found necessary to coat said base or preferably to saturate the same with moisture excluding material and, in practice, I have found asphalt or material of an asphaltic nature suitable for this purpose. It is found desirable to protect the floor covering at the top surface from wear of the feet and at its under surface from wear against or sticking to the floor on which the covering is placed. As the material of the body or base, at this stage, practically consists of a large proportion of asphaltic material carried by the fibrous sheet it is of course desirable that any subsequent operation should not effect the undue softening of the asphaltic material while it is also

desirable that the backing coating should be so applied to the surface of said base or body as in some cases to partially enter the interstices between the fibers or anchor itself 5 to the fibers and also that said backing coating when applied should present a comparatively smooth appearance. It is therefore preferred to apply the material in a condition rendered fluid by heat and to use material which will set or cool quickly and 10 will not thereafter become sticky and that the asphaltic material does not have an opportunity to become soft. In carrying out this step in my invention I have found, 15 after a series of experiments, that wax preferably of a hard and high melting nature can be used for this backing coating and I have found that Montan wax, a material manufactured from a particular kind of 20 coal, is effective as it does not retain heat to any material degree and when applied to the surface of the fibrous material as a thin coating at a temperature of about two hundred seventy five degrees, it cools or 25 hardens, at atmospheric temperature of 70 degrees, in a period of time so short as to be practically negligible while its nature is such that it does not readily flux with the

asphalt. When cool this backing coating is not unduly brittle but is tough and somewhat pliable and thereafter does not become sticky. In order to make this coating more ornamental it may be colored by the addition of suitable pigment. 30

I am aware that paraffin and similar 35 waxes have been applied as coatings to papers and I do not intend to claim such material.

Having thus described my invention I 40 claim as new and desire to secure by Letters Patent—

Floor covering comprising an elastic fibrous waterproofed base having a backing coating of hard Montan wax into which is received loose fibers of said waterproof material and constitutes a hard layer against which said elastic material may be compressed, and a top layer of paint applied directly to said elastic base and of a thickness and hardness adapted to distribute an 45 50 impact pressure thereon throughout a considerable area of said base.

CHARLES S. BIRD.

Witnesses:

MILLARD M. RINES,  
WALTER M. PAINE.